

## UNITED STATES PATENT OFFICE

2,129,554

## TANNING MATERIAL

Alfred Russell and John W. Copenhaver, Philadelphia, Pa., assignors to Rohm & Haas Company, Philadelphia, Pa.

No Drawing. Application October 30, 1937,  
Serial No. 172,043

12 Claims. (Cl. 149—5)

This invention relates to the production of new synthetic tanning materials that may be used in tanning skins, to retain leather made with other tanning materials, and to bleach and brighten chrome leather.

In our copending application Serial No. 161,066 filed August 26, 1937, it is shown that excellent tanning materials especially useful for bleaching chrome leather can be made by condensing a dihydroxy diaryl sulfone with formaldehyde. In copending application, Serial No. 172,042, filed on even date herewith, it is shown that the tanning and bleaching properties of these sulfone sulfonate-formaldehyde condensates can be improved by co-condensing urea and the sulfone-sulfonate with formaldehyde. We have also found that a similar improvement is obtainable if instead of starting with the sulfonated dihydroxy diaryl sulfone the unsulfonated material is reacted with urea and formaldehyde and the resulting water insoluble condensate dispersed in an aqueous solution of an aromatic sulfonic acid, such as naphthalene sulfonic acid. When applied to the bleaching of chrome tanned leather these materials give a rapid and intensive surface retannage and an improved quality white leather that has a remarkable resistance to sunlight.

In making the condensate the reaction is carried out on the acid side of neutrality, preferably in concentrated hydrochloric acid or sulfuric acid of equivalent strength. The dihydroxy diarylsulfone and urea may be dissolved in a strong aqueous solution of acid, the solution heated to a temperature at which formaldehyde condenses readily with the sulfone and the urea, and the formaldehyde added slowly while the mixture is being vigorously stirred. After all the formaldehyde is added, heating at the boiling point of the solution with reflux of vaporized material is continued until reaction is complete. If desired, the formaldehyde may be added to the cold solution of the sulfone and urea.

The relative proportion of urea, sulfone and formaldehyde that may be used varies over a wide range. The best ratio we have found is two molecular equivalents each of formaldehyde and sulfone to one molecular equivalent of urea. These ratios we believe give on condensation a molecule having the formula



wherein the R's are similar or dissimilar dihydroxy diaryl sulfone groups attached to the

methylene groups by nuclear carbon atoms. Reducing the quantity of urea reduces the amount of this material in the final condensate and accordingly while permissible is not recommended. The formaldehyde may likewise be reduced, particularly if less than the above stated amount of urea is used. However, there should be used one mol. of formaldehyde for each two mols of sulfone plus one mol. of formaldehyde for each mol. or urea. Increasing the ratio of urea and formaldehyde leads to the formation of more complicated molecules but up to four mols of formaldehyde and up to two mols of urea to two mols of sulfone may be used.

The tanning solution is prepared by adding the desired amount of the water insoluble condensate to an aqueous solution of naphthalene sulfonic acid and vigorously stirring, preferably while heating the mixture. Heating to aid dispersion of the condensate is unnecessary but substantially reduces the time required to obtain uniform and complete solution or dispersion of the material.

The following examples are given to illustrate the preparation of the new tanning materials. The conditions given are those we believe best suited for the purpose but it should be understood that these examples may be substantially departed from without departing from the invention. In these examples the parts given are parts by weight.

*Example 1.*—50 parts of 4:4' dihydroxy diphenyl sulfone was suspended in 300 parts of 36% aqueous hydrochloric acid containing 6 parts of urea and the suspension heated with vigorous stirring to 98–100° C. 20 parts of 30% aqueous formaldehyde was added slowly over 5 minutes and the whole maintained at a temperature of 98–100° C. under reflux with vigorous stirring for 2 hours. At this time an insoluble resin had separated. It was removed from the aqueous layer, washed twice with boiling water, and dried. 25 parts of this resinous material was added to a solution of 50 parts naphthalene sulfonic acid in 20 parts of water and the mixture heated with brisk stirring at 120° C. until complete solution was obtained and the product was stable to indefinite dilution with water. The reaction mixture was diluted to a final mass of 200 parts with water. This solution may be used directly for tanning or it may, if so desired, be partially neutralized with alkali first and then applied to tanning.

*Example 2.*—50 parts of 4:4' dihydroxy diphenyl sulfone was suspended in a solution of

100 parts 98% sulfuric acid dissolved in 175 parts of water containing 6 parts of urea. The suspension was heated to the boiling temperature under reflux and 20 parts of 30% aqueous form-  
 5 aldehyde added. The whole was maintained at the boiling temperature for 2 hours. At the end of this time the precipitated resin was collected, washed twice with boiling water, dried, and dispersed in a solution of naphthalene sulfonic acid  
 10 and water using the quantities and method de-  
 scribed in Example 1.

The dihydroxy diphenyl sulfone used in these examples can be replaced with equivalent quantities of other dihydroxy diaryl sulfones such as  
 15 the tolyl homologue.

While the new tanning materials can be used for tanning raw skins or retanning skins tanned by other materials, they are of particular value in bleaching chrome tanned leather. To illus-  
 20 trate this use, the following example is given.

*Example 3.*—100 pounds of fully tanned chrome calfskin is drummed for an hour at 140° F. with 150 pounds of water and ten pounds, or other suitable quantity, of the tanning material pre-  
 25 pared as described in the preceding example. The stock is now washed with water till it shows a pH of 4-4½ when it may be oiled and finished in any recognized manner. The leather so produced has a white surface of remarkable re-  
 30 sistance to the action of strong sunlight.

We claim:

1. The process of preparing a synthetic tanning material which comprises co-condensing a dihydroxy diaryl sulfone and urea with formalde-  
 35 hyde in strong acid solution and dispersing the resinous material obtained in an aqueous solution of an aromatic sulfonic acid.
2. The process of preparing a synthetic tanning material which comprises co-condensing a dihydroxy diphenyl sulfone and urea with formalde-  
 40 hyde in strong acid solution and dispersing the resinous material obtained in an aqueous solution of an aromatic sulfonic acid.
3. The process of preparing a synthetic tan-  
 45 ning material which comprises co-condensing 4:4' dihydroxy diphenyl sulfone and urea with formaldehyde in strong acid solution and dispersing the resinous material obtained in an aqueous solution of naphthalene sulfonic acid.
- 50 4. The process of preparing a synthetic tanning material which comprises co-condensing substantially two molecular equivalents of a dihydroxy diphenyl sulfone and substantially one molecular equivalent of urea with substantially two molecular equivalents of formaldehyde and

dispersing the resinous material obtained in an aqueous solution of an aromatic sulfonic acid.

5. The process of preparing a synthetic tan-  
 ning material which comprises co-condensing substantially two molecular equivalents of a di-  
 5 hydroxy diphenyl sulfone and substantially one molecular equivalent of urea with substantially two molecular equivalents of formaldehyde and dispersing the resinous material obtained in an aqueous solution of naphthalene sulfonic acid. 10

6. A synthetic tanning material which is a joint condensation product of a dihydroxy diaryl sulfone and urea with formaldehyde dispersed in an aqueous solution of an aromatic sulfonic acid.

7. A synthetic tanning material which is a joint condensation product of a dihydroxy diaryl sulfone and urea with formaldehyde dispersed in an aqueous solution of naphthalene sulfonic acid. 15

8. A synthetic tanning material which is a joint condensation product of 4:4' dihydroxy di-  
 20 phenyl sulfone and urea with formaldehyde dispersed in an aqueous solution of naphthalene sulfonic acid.

9. A synthetic tanning material which is a joint condensation product of substantially two molecular equivalents of a dihydroxy diphenyl sulfone and substantially one molecular equivalent of urea with substantially two molecular equivalents of formaldehyde dispersed in an aqueous solution of an aromatic sulfonic acid. 25

10. A synthetic tanning material which is a joint condensation product of substantially two molecular equivalents of a dihydroxy diphenyl sulfone and substantially one molecular equivalent of urea with substantially two molecular equivalents of formaldehyde dispersed in an aqueous solution of naphthalene sulfonic acid. 30

11. In a process of making leather the improvement which comprises treating a chrome tanned leather with a joint condensation product of a dihydroxy diphenyl sulfone, urea and formaldehyde dispersed in an aqueous solution of naphthalene sulfonic acid. 35

12. In a process of making leather the improvement which comprises treating a chrome tanned leather with a joint condensation product of substantially two molecular equivalents of a dihydroxy diphenyl sulfone, substantially one molecular equivalent of urea, and substantially two molecular equivalents of formaldehyde dispersed in an aqueous solution of naphthalene sulfonic acid. 40 45 50

ALFRED RUSSELL.

JOHN W. COPENHAVER. 55

CERTIFICATE OF CORRECTION.

Patent No. 2,129,554.

September 6, 1938.

ALFRED RUSSELL, ET AL.

It is hereby certified that error appears in the printed specification of the above numbered patent requiring correction as follows: Page 1, first column, line 24, for the article "the" second occurrence, read of; line 33, for "diarylsulfone" read diarylsulfone; and second column, line 10, for "or" read of; page 2, first column, line 43, claim 2, for the syllable and words "tion of an aromatic" read lution of naphthalene; and that the said Letters Patent should be read with this correction therein that the same may conform to the record of the case in the Patent Office.

Signed and sealed this 10th day of January, A. D. 1939.

(Seal)

Henry Van Arsdale  
Acting Commissioner of Patents.